

July 10, 1934.

J. H. DE BOER ET AL

1,966,236

PHOTO ELECTRIC TUBE

Filed Nov. 28, 1931



INVENTORS

JAN HENDRIK DE BOER AND  
MARTEN CORNELIS TEVES

BY

*H.S. Snover*  
ATTORNEY

## UNITED STATES PATENT OFFICE

1,966,236

## PHOTO ELECTRIC TUBE

Jan Hendrik de Boer and Marten Cornelis Teves,  
Eindhoven, Netherlands, assignors to Radio  
Corporation of America, a corporation of Dela-  
ware

Application November 28, 1931, Serial No. 577,740  
In Germany December 6, 1930

5 Claims. (Cl. 250—27.5)

In the main patent specification No. 452,785 it has been proposed to provide the photo-electric substance of the light sensitive electrode of a photo-electric tube on a layer containing a chemical compound and electrically-conducting particles. As set forth in the said specification, these particles may be particles of the photo-electric substance and it is advisable to provide in the layer, in addition to the particles of said photo-electric substance, particles of another conducting material. By a photo-electric substance is meant hereinafter a substance which emits electrons when exposed to radiation.

The invention has for its object to increase the sensitivity of such a photo-electric tube i. e. the current produced in the tube due to a determined exposure of the photo-electric electrode to radiation.

A photo-electric tube according to the invention contains a photo-electric metal present on a layer containing, in addition to particles of said metal and to particles of another conducting substance, particles of the oxide of the photo-electric metal. The film of photo-electric metal present on the said layer is preferably made very thin; it has for example, a thickness of one or a few atoms. The layer supporting this photo-electric metal i. e. the above-described mixed layer, should preferably be thick, for example thicker than 100 molecules.

As the photo-electric metal use is preferably made of the alkali metals although other substances, for example the alkaline earth metals such as barium may be utilized as well.

In the manufacture of such a photo-electric tube one preferably proceeds as follows. A layer of metal oxide, for example silver oxide, is first produced within the tube, which may be effected by oxidizing a metal layer produced, for example, by evaporation in a vacuum. The metal oxide layer may also be obtained, however, in another manner, for example by evaporating a metal oxide present on an incandescent body arranged within the tube. After the formation of the metal oxide layer and, if desired, after the exhaustion of the tube, an excess of photo-electric metal, for example of alkali-metal, is introduced into the tube which while not connected to a vacuum pump is heated to such a temperature that the metal oxide is reduced and the oxide of the photo-electric metal, for example alkali oxide, is formed. The excess of photo-electric metal is given the opportunity of penetrating into the produced mixture of particles of the reduced metal and particles of the oxide of

the photo-electric metal and for this purpose it is advantageous slightly to heat the tube, for example to about 100° C. During this heating a film of alkali metal deposits on the layer produced.

In reducing the metal oxide care should be taken to prevent the tube from being heated to such an extent that the oxide of the photo-electric metal decomposes or volatilizes or that the metal particles produced clot together.

In order that the invention may be clearly understood and readily carried into effect it will be explained more fully with reference to the accompanying drawing which represents, by way of example, a photo-tube according to the invention. In the drawing:

Figure 1 is a section of this photo-electric tube and

Figure 2 represents a detail thereof.

The photo-electric tube shown in Figure 1 has a spherical wall 1 to which is sealed a tube 2 provided with a stem 3 which carries the electrode 4 of the photo-electric tube. As distinctly appears from Figure 2 this electrode consists of a nearly closed metal ring the ends of which are connected to current supply wires 5 and 6. The wall 1 is coated with a silver layer 7 which is electrically connected to a current supply wire 8. The silver layer 7 is covered with a layer 9 consisting of intimately mixed silver particles, caesium particles and caesium oxide particles, this intermediate layer 9 being provided with a caesium film 10.

In manufacturing the tube, first a silver layer is formed on the wall. For this purpose, some silver may be secured to the electrode 4 prior to the arrangement of the latter in the tube, said quantity of silver being evaporated by heating the electrode 4 after the tube has been exhausted, which may be effected with the aid of a vacuum pump connected to the exhaust tube 11. The evaporated silver settles on the wall of the tube, a portion 12 of said wall being kept free from silver deposit by means of a screen not shown in the drawing. This portion 12 constitutes the window through which during operation the rays of light penetrate into the tube. The silver layer may also be formed in other ways than by evaporation in a vacuum, for example by precipitation from a silver compound.

After the silver layer has been formed, oxygen, for example in the form of air, is admitted into the tube and an electric discharge is established between the electrode 4 and the silver layer, owing to which the surface of the silver layer is

oxidized. The oxidation should preferably be continued until a rather thick layer of silver oxide of uniform structure has been formed.

Subsequently, the tube is exhausted again and 5 shut off from the pump whereupon caesium is introduced in excess into the tube, for example by distillation from a receptacle (not shown in the drawing) which is connected to a tube 13. The caesium may also be developed within the tube 10 for example by heating a mixture of a caesium compound and a suitable reducing agent. When after the introduction of the caesium into the tube the latter is heated to about 200° C., the silver oxide is reduced and caesium oxide is formed. 15 Care should be taken, that during this heating operation the tube is not connected to the vacuum pump as otherwise the caesium would be withdrawn from the tube. Furthermore, the temperature must not be raised too much. If, for 20 example, the tube would be heated to 250° C., the caesium oxide, which has the composition Cs<sub>2</sub>O, would volatilize and at a higher temperature it would even be decomposed. Besides, at 25 that high temperature the silver particles would melt together so that they would no longer be present in the layer in a finely divided state.

During and after the formation of the mixture of silver particles and caesium oxide the excess of caesium is given the opportunity of penetrating 30 into the mixture formed. This penetration can be facilitated by heating the tube, for example to 100° C., the tube being during this heating operation not in communication with a vacuum pump. A layer is thus obtained which contains 35 silver particles, caesium particles and caesium oxide particles in a mixed state.

Part of the caesium settles as a thin film on this intermediate layer. If within the tube there should still be some free caesium this may be removed from the tube, if desired, by connecting 40 the latter to a vacuum pump and by exhausting cold. Alternatively, it is possible to connect the tube to a side-tube which is subsequently cooled and sealed off, or to introduce into the tube a 45 substance adapted to absorb the excessive caesium, for example finely divided carbon. Use may also be made of a chemical compound capable of taking up the excessive caesium, for example of lead oxide. For this purpose for example 50 the stem of the tube may be made of lead glass.

It is evident that the photo-electric substance may consist not only of caesium but also of other alkali metals or other substances, for example barium, while the intermediate layer may also 55 contain particles of a metal other than silver. The tube is preferably used as a high vacuum tube but it is also possible to provide it with a gaseous filling.

The photo-electric tube according to the invention has a very great sensitivity. In high-vacuum tubes it is possible for example, to obtain currents of 40 micro-amperes per lumen. These are currents being about ten times as strong as those reached in the high-vacuum tubes 65 according to the main patent. Besides, the tubes can be made so as to be perfectly reproducible so that they are suitable for mass-production.

What we claim is:

1. In the manufacture of a photoelectric tube

70

comprising an evacuated envelope enclosing an anode and a cathode having a surface which contains silver, the process which consists in oxidizing the silver containing surface of said cathode, evacuating said envelope, producing in said evacuated envelope an atmosphere of alkali metal vapor, heating said cathode in said atmosphere to reduce some of the silver oxide on the surface of said cathode to metal without preventing the formation of oxide of the alkali metal on said surface, holding said cathode at a temperature slightly below the vaporizing point in said envelope of the alkali metal for a time sufficient to permit said alkali metal to deposit from said atmosphere on the surface of said cathode and penetrate said surface, and removing the excess of alkali metal vapor. 80 85 90

2. The method of producing a light sensitive coating on a silver surfaced cathode of a photoelectric tube having an envelope enclosing said cathode, which consists in oxidizing the surface of said cathode, evacuating and temporarily sealing the envelope of the tube, producing in the sealed evacuated envelope an atmosphere containing alkali metal vapor, heating said cathode 100 in said atmosphere to a temperature sufficient to reduce to particles of silver some of the silver oxide on the surface of said cathode and insufficient to vaporize oxide of said alkali metal from said surface, lowering the temperature of said cathode to slightly below the temperature at which the alkali metal deposits on said cathode from said alkali metal vapor atmosphere, holding said cathode at said lower temperature for a time to permit some penetration of said surface by said alkali metal, and removing the excess alkali metal vapor. 105 110

3. In the manufacture of a photoelectric tube comprising an evacuated envelope enclosing a cathode having a surface which is predominantly 115 silver, the method of rendering said cathode light sensitive which consists in oxidizing said cathode surface, producing in said evacuated envelope an atmosphere containing caesium vapor, heating said cathode in the presence of said 120 atmosphere to about 200° C. and below 250° C. until some of the oxidized silver is reduced to finely divided metal, maintaining said cathode at about 100° C. to produce a thin film of caesium on said surface, and removing the excess of 125 caesium. 130

4. A photoelectric tube comprising an envelope enclosing an anode and a cathode comprising a metal base having on its surface a mixture of particles of the metal of the base, of an alkali metal, and of oxide of said alkali metal in the form of a thin layer, and a film of said photoelectric metal on said layer. 140

5. A photoelectric tube comprising an envelope enclosing an anode and a cathode comprising a 135 silver plate having its surface coated with a relatively thick layer of a mixture of finely divided silver, of caesium oxide, and of particles of caesium, and a relatively thin film of caesium on said layer. 140

JAN HENDRIK DE BOER.  
MARTEN CORNELIS TEVES.

145

75

150